

# United States Patent

[19]

Magne et al.

[11] 3,873,457

[45] \*Mar. 25, 1975

[54] **N-SUBSTITUTED FATTY ACID AMIDE LUBRICANTS**

[75] Inventors: **Frank C. Magne; Robert R. Mod; Gene Sumrell**, all of New Orleans, La.

[73] Assignee: **The United States of America as represented by the Secretary of Agriculture**, Washington, D.C.

[\*] Notice: The portion of the term of this patent subsequent to July 17, 1990, has been disclaimed.

[22] Filed: **Feb. 21, 1973**

[21] Appl. No.: **334,318**

## Related U.S. Application Data

[63] Continuation-in-part of Ser. No. 176,734, Aug. 31, 1971, Pat. No. 3,746,644.

[52] **U.S. Cl.** ..... **252/47.5, 252/48.4; 252/48.6**

[51] **Int. Cl.** ..... **C10m 1/38**

[58] **Field of Search** ..... **252/48.2, 48.4, 48.6**

[56]

## References Cited

### UNITED STATES PATENTS

|           |         |                        |            |
|-----------|---------|------------------------|------------|
| 3,166,504 | 1/1965  | Krukziener et al. .... | 252/48.6 X |
| 3,400,139 | 9/1968  | Calhoun.....           | 252/48.6 X |
| 3,733,275 | 5/1973  | Magne et al. ....      | 252/46.7 X |
| 3,746,644 | 7/1973  | Magne et al. ....      | 252/47.5   |
| 3,766,069 | 10/1973 | Hotten.....            | 252/48.6   |

*Primary Examiner*—Patrick P. Garvin

*Assistant Examiner*—Andrew H. Metz

*Attorney, Agent, or Firm*—M. Howard Silverstein; Max D. Hensley

[57]

## ABSTRACT

This invention relates to N-acylmorpholines and N-mono and N,N-disubstituted fatty acid amides and to similar derivatives of epithioamides which are useful as base and extreme pressure lubricants and additives.

**41 Claims, No Drawings**

**N-SUBSTITUTED FATTY ACID AMIDE  
LUBRICANTS**

A non-exclusive, irrevocable, royalty-free license in the invention herein described, throughout the world for all purposes of the United States Government, with the power to grant sublicenses for such purposes, is hereby granted to the Government of the United States of America.

This application is a continuation-in-part of Ser. No. 176,734 filed Aug. 31, 1971, said 176,734 now U.S. Pat. No. 3,746,644.

This invention relates to certain compounds which are N-fatty acyl derivatives of primary and secondary amine and N-substituted acyl derivatives of primary and secondary amines which have exhibited utility as base lubricants, extreme pressure lubricants or lube additives. More particularly, this invention relates to N- and NN-disubstituted long chain aliphatic amides the acyl component of which is a normal, branched, or substituted alkenoic or alcanoic acyl group containing from 16 to 22 carbon atoms the amide nitrogen of which may be derived from an alkyl amine, dialkyl amine, alkyl-alkoxyalkylamine, dialkoxyalkylamine or nitrogen heterocyclic. Typical amines are butylamines, dibutylamines, N-methyl-alkoxyethyl amine, diethoxyethyl amine, and morpholine. The acyl substituent referred to may be divalent sulfur or pentavalent phosphorous.

We have discovered that many of the simple N-alkyl and N,N-dialkyl or N-alkyl-N-alkoxyalkyl amides of the C<sub>16</sub> to C<sub>22</sub> alkeneoic or alcanoic fatty acids are good base lubricants. We have further discovered that the introduction of divalent sulfur into the fatty acid moiety imparts excellent extreme pressure lubricant characteristics to such compounds. We have also found this to be true for glycerides and simple esters even when the divalent sulfur substituent group is in the alkyl moiety. In particular we have found the epithio group

-C - C -  
's'

to be most effective. We have also observed that the introduction of both hydroxy and alkyl phosphato groupings alpha to each other also imparts extreme pressure lubricant characteristics to the compound.

In addition it was noted that the above hydroxyphosphato compound and its mercapto analog N-[9(10)-mercapto-(9)10-dibutylphosphato]stearamide were effective antiwear compounds and additives.

Included among the specific compounds operable as base lubricants are N-methyl-N-butyloleamide, N-ethoxyethoxyethoxy propyoleamide, N-ethoxyethoxy propyoleamide, N-methoxyisopropyoleamide, N-methoxyethoxyoleamide. Compounds showing particular promise as extreme pressure lubricants or additives are N,N-dibutyl-9,10-epithiostearamide, N,N-dibutyl-9,10-12, 13-diepithiostearamide, 9,10-epithiostearoyl morpholine, N-ethoxyethoxyethoxypropyl-9,10-epithiostearamide, N-9,10-12,13-diepithiostearoylmorpholine and N-[9(10)-hydroxy-9(10)-dibutylphosphato]stearamide, as well as epithioated soybean oil, an epithioated glyceride, 9,10-epithiostearyl 9,10-epithiostearate and epithioated (o)oba oil both simple alkyl esters, and other ester types as 1,3-bis(9,10-epithiostearoyloxy)propane,

2-ethoxyethyl 9,10-epithiostearate, 2-(2-ethoxyethoxy)ethyl 9,10-epithiostearate, 2-ethoxyphenyl 9,10-epithiostearate, 9,10-epithiostearyl pentachlorostearate, 4-methoxyphenyl 9,10-epithiostearate, 9,10-epithiostearoyl terminated sebacic acid-1,3-propanediol polyester, N-methyl-N-[2-(9,10-epithiostearoyloxy)ethyl]-9,10-epithiostearamide, N-[2-(9,10-epithiostearoyloxy)ethyl]-9,10-epithiostearamide, 1,3-bis epithiostearoyl imidazolidine, 1,3-bis epithiostearoyl hexahydropyrimidine.

Compounds showing particular promise as antiwear additives are N,N-dibutyl-[9(10)-hydroxy-(9)10-dibutylphosphato]stearamide and N,N-[9(10) mercapto-(9)10-dibutylphosphostearoyl]morpholine.

**EXAMPLE 1**

**N-Methyl-N-butyloleamide**

100 grams (0.33 mole) of oleoyl chloride was added dropwise and with stirring to a mixture of 29 grams (0.33 mole) of N-methyl-N-butylamine and 27 grams (0.33 mole) of pyridine. Stirring was continued until the heat of reaction subsided. The solid pyridine hydrochloride was filtered off and the filtrate was washed successively with aqueous HCl and water until acid free. It was dried stripped, percolated through an activated alumina column, and the product removed from the percolate by stripping off the solvent. Analysis of the product: Percent C, 78.87 (theory 78.63; percent H, 13.02 (theory 12.82); percent N, 3.96 (theory 3.99).

**EXAMPLE 2**

**N,N-dibutyloleamide**

35 This material was prepared by the procedure of Example 1 from 100 grams (0.33 mole) of oleoyl chloride 42.5 grams (0.33 moles of di-n-butylamine and 27 grams (0.33 mole) pyridine. Analysis of the product: Percent C, 78.94 (theory 79.25); percent H, 13.16 (theory 13.06); percent N, 3.44 (theory 3.56) confirm the preparation.

**EXAMPLE 3**

**Ethoxyethoxyethoxy propyoleamide**

45 This material was prepared by the procedure of Example 1 from 100 grams (0.33 mole) of oleoyl chloride, 73.0 grams (0.33 mole) ethoxyethoxyethoxypropylamine and 27.0 grams (0.33 mole) pyridine. Analysis of percent C, 71.84 (theory 72.04); H, 11.80 (theory 11.80), and N, 2.96 (theory 2.90) confirm the preparation.

**EXAMPLE 4**

**Ethoxyethoxypropyoleamide**

55 This material was prepared by the procedure of Example 1 from 100 grams (0.33 mole) of oleoyl chloride, 58.3 grams (0.33 mole) ethoxyethoxypropylamine and 27.0 grams (0.33 mole) of pyridine. Analyses of percent C, 71.45 (theory 73.80); percent H, 11.87 (theory 12.07); and percent N, 2.92 (theory 3.18) confirm the preparation.

**EXAMPLE 5**

**Methoxyisopropyoleamide**

65 This material was prepared by the procedure of Example 1 from 100 grams (0.33 mole) of oleoyl chlo-

ride, 29.3 grams (0.33 mole) methoxyisopropylamine and 27.0 grams (0.33 mole) pyridine. Analysis of percent C, 73.15 (theory 74.99); percent H, 12.01 (theory 11.93); and percent N, 3.67 (theory 3.97) confirm the preparation.

#### EXAMPLE 6

##### Methoxyethyloleamide

This material was prepared by the procedure of Example 1 from 100 grams (0.33 mole) of oleoyl chloride, 24.4 grams (0.33 mole) of methoxyethylamine and 27.0 grams (0.33 mole) pyridine. Analysis of percent C, 73.08 (theory 74.55); percent H, 11.98 (theory 11.83); and percent N, 3.31 (theory 4.14) confirm the preparation.

#### EXAMPLE 7

##### Oleoylmorpholine

This material was prepared by the procedure of Example 1 from 100 grams (0.33 mole) of oleoyl chloride, 28.7 grams (0.33 mole) of morpholine and 27.0 grams (0.33 mole) of pyridine.

#### EXAMPLE 8

##### N,N-dibutyloleamide

This product was prepared following the exact procedure of Example 2 except for the substitution of oleoyl chloride by linoleoyl chloride.

#### EXAMPLE 9

##### N,N-dibutyl-9,10-epithiostearamide

120 grams (0.30 mole) of N,N-dibutyloleamide was epoxidized by the addition with stirring of 62.0 grams (0.36 mole) of meta-chloroperbenzoic acid in 630 ml of chloroform. Reaction was continued for 1 hour beyond final addition and the excess peracid destroyed by a small amount of a 10% solution of  $\text{Na}_2\text{SO}_3$ . The meta-chlorobenzoic acid was removed by a  $\text{NaHCO}_3$  wash, followed by water washing. The  $\text{CHCl}_3$  solution was then dried with anhydrous  $\text{Na}_2\text{SO}_4$  and the  $\text{CHCl}_3$  stripped off to recover the product N,N-dibutyl-9,10-epoxystearamide, oxirane content 3.45% (theory 3.91%). 100 grams (0.24 mole) of this product was added to a well stirred slurry of 55.7 g (0.75 moles) of thiourea and 89.5 g (0.72 moles) of benzoic acid in acetone. Stirring was continued for 3 hours beyond the terminal addition whereupon the benzoic acid was washed out with 38.8 g (0.36 mole) of  $\text{Na}_2\text{CO}_3$  and the organic product extracted with hexane. The organic phase extract was dried and stripped to recover the product N,N-dibutyl-9,10-epithiostearamide containing 6.41% sulfur (theory 6.67%).

#### EXAMPLE 10

##### N-(9,10-epithiostearoyl)morpholine

This product was prepared by the exact procedure described in Example 9 except for the substitution of oleylmorpholine for the N,N-dibutyloleamide of Example 9. Analysis of product showed percent C, 71.22 (theory 69.34); percent H, 11.22 (theory 10.77); percent N, 3.66 (theory 3.68); percent S, 3.44 (theory 7.80).

#### EXAMPLE 11

##### N,N-dibutyl-9,10-9,10-12,13-diepithiostearamide

This product was prepared following the procedure described in Example 9 except for the replacement of the N,N-dibutyloleamide of Example 9 by N,N-dibutyllinoleamide, and a doubling of the molar ratios of all reagents. The product analyzed as follows: percent C, 69.64 (theory 68.57); percent H, 10.93 (theory 10.76); percent N, 3.10 (theory 3.07); percent S, 11.7 (theory 14.06).

#### EXAMPLE 12

##### N-Ethoxyethoxyethoxypropyl-9,10-epithiostearamide

To 166 g of N-ethoxyethoxyethoxypropyl oleamide, Example 3, was added dropwise and with stirring 73.8 g of m-chloroperbenzoic acid in 800 ml of  $\text{CHCl}_3$ . The spent m-chloroperbenzoic acid was removed with 10% aqueous  $\text{NaHCO}_3$  and the epoxide recovered by drying and stripping off the  $\text{CHCl}_3$ . 171 g of this epoxide was added dropwise to a slurry of 56 g thiourea in 1,000 ml of acetone and the concurrent addition of 43.4 g of glacial acetic acid and the reaction mixture stirred for 3 hours. The glacial acetic acid was neutralized with  $\text{Na}_2\text{CO}_3$  and the episulfide, N-ethoxyethoxyethoxypropyl-9, 10-epithiostearamide, extracted with Skellysolve B and washed, dried, and stripped. Its elemental analysis was C = 67.1 (66.52), H = 11.42 (10.88), N = 2.67 (2.87), S = 2.29 (6.57).

#### EXAMPLE 13

##### N-Ethoxyethoxyethoxypropyl-9(10)mercaptopstearamide

173 g of N-ethoxyethoxyethoxypropyleamide in  $\text{CCl}_4$  was treated in the cold with a  $\text{CCl}_4$  solution containing 60.9 g of bromine. Any unreacted bromine was removed by a thiosulfate wash. 140 g of the resulting dibromo compound was added dropwise to a well stirred solution of 72 g of  $\text{Na}_2\text{S} \cdot 9\text{H}_2\text{O}$  in dimethylsulfoxide maintained at 80°C. Stirring was continued at 80°C for 3 hours. Water was added and the reaction product was extracted with hexane; washed, dried, and stripped. Elemental analysis of the product was C = 66.3 (66.5); H = 11.1 (10.9), N = 2.7 (2.9), S = 4.4 (6.8).

#### EXAMPLE 14

##### N,N-Dibutyl-9(10)[dibutylphosphono]stearamide

100 g of N,N-dibutyloleamide, Example 2, 148 g of dibutyl phosphite, and 1.29 of benzoyl peroxide catalyst were heated at 115°C for 3-1/2 hours. Additional units of 1.29 g of benzoyl peroxide was added after the first and second hours of reaction time. The excess dibutyl phosphite was then removed by distillation at reduced pressure, 0.45 mmHg. The stillpot contents showed strong adsorption bonds at 8,9,3, and 9.7 microns characteristics of the phosphonate group. The elemental analysis was C = obs 71.46 (69.50), H = obs 12.42 (11.92), N = obs 2.20 (2.38), P = obs 4.24 (5.28) percent respectively.

#### EXAMPLE 15

##### N-9,10-12,13-diepithiostearoylmorpholine

This product was prepared by the same procedure described in Example 9 except for the substitution of linoleoyl morpholine for the N,N-dibutyloleamide of

Example 8 and the doubling of molar proportions of the m-chloroperbenzoic acid in the epoxidation step and the thiourea and benzoic acid in the "epithioation" step. The elemental analysis was C = obs 68.89 (63.92), H = obs 10.26 (9.44), N = obs 3.29 (3.38), S = obs 4.00 (15.49) percent respectively.

#### EXAMPLE 16

##### N,N-Dibutyl-[9(10)-hydroxy-(9)10-dibutylphosphato]stearamide

44.7 g of dibutylhydrogen phosphate was added to 182.2 g of N,N-dibutyl-9,10-epoxystearamide at 90-95°C with stirring. Reaction conditions were continued for 3-½ hours after termination of the addition. The reaction product was dissolved in commercial hexane and the unreacted dibutyl hydrogen phosphate neutralized and washed out with portions of aqueous 10% NaHCO<sub>3</sub> followed by several water washes. Acidulation of the hexane phase with diluted HCl followed by several water washes, drying and stripping, yielded the product. Elemental analysis was, C = obs 66.56 (65.91), H = obs 11.04 (11.30), N = obs 2.90 (2.26), P = obs 3.04 (4.20).

#### EXAMPLE 17

##### N-[9(10)mercapto-(9)10-dibutylphosphatostearoyl]-morpholine

12 g of dibutylhydrogen phosphate was added dropwise with stirring to 51.0 g of (9,10-epithiostearoyl)-morpholine, the preparation of Example 10, at 85°-90°C and the heating and stirring continued for 3 hours beyond the terminal addition. The reaction product was dissolved in commercial hexane and any excess or unreacted



was neutralized and washed out with aqueous 10% NaHCO<sub>3</sub>. The hexane extract was washed several times with water dried and stripped. The elemental analysis of the product was C = obs 66.74 (69.36), H = obs 10.69 (11.05), N = obs 2.89 (3.32), S = obs 3.27 (2.17), P = obs 1.68 (2.10) percent respectively.

#### EXAMPLE 18

##### 9,10-Epithiostearyl 9,10-epithiostearate

140 grams of a commercial oleic acid (Emersol 233LL), 119 g of commercial oleyl alcohol (Aldol 85) and 50 ml of toluene were refluxed in the presence of 3 g of p-toluene sulfonic acid for 24 hours, with a continual removal of the water of reaction by a Dean-Stark trap. The reaction mixture was freed of p-toluene sulfonic acid and any unreacted fatty acid by repeated washings with aqueous NaHCO<sub>3</sub> solution. The product, oleyl oleate, was isolated by stripping off the toluene from the Na<sub>2</sub>SO<sub>4</sub> dried mixture.

The oleyl oleate was converted to 9,10-epoxystearyl 9,10-epoxystearate by treatment with a chloroform solution of meta-chloroperbenzoic acid containing 5% excess of per acid over that theoretically necessary to epoxidize the two double bonds present per mole of oleyl oleate. The product 9,10-epoxystearyl 9,10-epoxystearate had an oxirane content of 4.99.

112 g of the 9,10-epoxystearyl 9,10-epoxystearate was converted to 9,10-epithiostearyl 9,10-epithioste-

rate by the dropwise addition of a 1-4 dioxane solution (300 ml dioxane) of the former over a 2-2-½ hour period to a vigorously stirred aqueous solution containing 34.2 g of thiourea in minimal water and 22.0 g of H<sub>2</sub>SO<sub>4</sub> as a 30% aqueous solution maintained at a temperature of 5°C.

#### EXAMPLE 19

##### Epithioated Soybean Oil

300 grams of a commercially available epoxidized soybean oil (oxirane content 7.1%) was dissolved in 500 ml of 1-4 dioxane and added dropwise over a 2 hour period to a vigorously stirred solution composed of 101.2 g of thiourea in minimal water and 65.0 g of H<sub>2</sub>SO<sub>4</sub> (the latter as a 30% aqueous solution), maintained at 5°C. After the addition was completed the reaction mixture was raised to 40°C and kept stirred for 2 hours as it cooled. 70.6 g of Na<sub>2</sub>CO<sub>3</sub> in the form of a 10% aqueous solution was added with stirring and the mixture warmed up to 40°C and stirring continued for 1 hour. The epithioated soybean oil was then extracted with 200 ml of benzene and the extract washed, dried, and the benzene stripped off. The recovered oil had a sulfur content of 6.97% as opposed to a theoretical value of 13.25% for total conversion of oxirane to thirane.

#### EXAMPLE 20

##### Epithioated Jojoba oil

125 g of jojoba oil (1 V = 83.6) was epoxidized by the addition of 133.0 g of m-chloroperbenzoic acid in 1,500 ml of CHCl<sub>3</sub> while maintaining a temperature of 20°-25°C to an oxirane content of 3.56%. The recovered product (131 g of epoxide) was converted to the epithio analog by its reaction with 30.9 g thiourea and 66.6 g of H<sub>2</sub>SO<sub>4</sub>, following the same reaction procedure described in Example 19. The reaction mixture was treated with 21.5 g of Na<sub>2</sub>CO<sub>3</sub> in 195 ml of H<sub>2</sub>O following the procedure of Example 19 and the epithio analog recovered as described in the previous example. The thirane content (epithiosulfur) was 2.31%. Complete conversion of oxirane to thirane should have given 6.87% sulfur.

#### EXAMPLE 21

##### 9,10-Epithiostearoyl terminated polyester of sebacic acid and 1,3-propane diol.

I. 190 g (0.82 moles) of dimethyl sebacate was added dropwise to a refluxing mixture of 110 g (1.44 moles) of 1,3-propane diol and 7.0 g of sodium methoxide in an apparatus equipped with a condenser, Dean-Stark trap and short Vigreux column intervening between trap and flask. Reaction was stopped when mixture became viscous and visible evolution of methanol was no longer observed. The alkoxide catalyst was killed with dilute hydrochloric acid and the polyester dissolved in diethyl ether was washed, the solution dried and stripped. The recovered product had a molecular weight of 493 and a hydroxyl content of 5.20%.

II. 144.6 g of oleyl chloride was added dropwise to 158 g of the product I in 38.0 g of pyridine and 100 ml of benzene with vigorous stirring. The crude reaction product was filtered, washed and dried and passed through two successive activated alumina columns using diethyl ether as the solvent system to remove any free acid.

III. 100 g of product II was epoxidized by the addition at 20°-25°C with stirring of 34.4 g of meta-chloroperbenzoic acid in chloroform. The epoxide product was processed and recovered as described in previous examples. The oxirane content of the product was 2.30%.

IV. The epoxy polyester III, 100 g, in 200 ml of dioxane was added dropwise over a 2-3 hour period to 6.4 g of thiourea in minimal water to which had been added 4.2 g of H<sub>2</sub>SO<sub>4</sub> as a 30% aqueous solution. The addition was carried out with vigorous stirring with the temperature maintained at +5°C. After the addition was complete the reaction mixture was warmed up to 40°C and stirred for 1-2 hours and allowed to cool and 4.7 g of Na<sub>2</sub>CO<sub>3</sub> in 50 ml of water added, the mixture again warmed up to 40°C with stirring. The product was then extracted with benzene, washed dried and stripped. Analysis showed a sulfur content of 1.1%.

#### EXAMPLE 22

I. N-[2-(9,10-epithiostearoyloxy)ethyl]-9,10-epithiostearamide. 150 g of oleoylchloride was added dropwise with stirring to 15.2 g of ethanolamine and 19.7 g of pyridine in 300 ml of benzene. The product N-(2-oleoyloxyethyl)oleamide was recovered in the usual manner.

II. The product I, 100 g, was epoxidized as described in preceding examples with 69.0 g of metachloroperbenzoic acid. The epoxide N-[2-(9,10-epoxystearoyloxy)ethyl]-9,10-epoxystearamide was produced in about a 50% yield. It had an oxirane content of 3.50%.

III. 112 g of the diepoxide II was added dropwise to a well stirred mixture of 59.6 g of thiourea and 95.6 g of benzoic acid in 500 ml of acetone at room temperature. After stirring for a total of 3 hours it was treated with 55.0 g of K<sub>2</sub>CO<sub>3</sub> in 600 ml of water. The product was extracted with Skelly B washed, dried, and stripped. The product whose principal component was N-[2-(9,10-epithiostearoyloxy)ethyl]-9,10-epithiostearamide gave the following analysis: C=69.24 (69.83), H = 10.66 (10.87), N = 1.97 (2.14), S = 6.50 (9.80). Calculated value in parentheses.

#### EXAMPLE 23

N-Methyl-N-[2-(9,10-epithiostearoyloxy)ethyl]-9,10-epithiostearamide.

I. 300 g of oleoyl chloride was added with stirring to 38.5 g of N-methylethanolamine and 39.5 g of pyridine in 200 ml of benzene. The product N-methyl-N-(2-oleoyloxyethyl)oleamide was recovered in the usual manner.

II. 125 g of I was epoxidized by the addition of 84.3 g of meta-chloroperbenzoic acid at 20°-25°C in CHCl<sub>3</sub>. The recovery and isolation and procedures were the same as described in preceding examples. The product composed principally of N-methyl-N-[2-(9,10-epoxystearoyloxy)ethyl]-9,10-epoxystearamide had an oxirane content of 4.74%.

III. 100 g of II was added dropwise over a 2-3 hour period to a slurry of 52 g of thiourea and 82.9 g of benzoic acid in 700 ml of acetone at room temperature. 200 ml of 10% Na<sub>2</sub>CO<sub>3</sub> was then added and the epithio compound recovered as in the preceding example. The product N-Methyl-N-[2-(9,10-epithiostearoyloxy)ethyl]-9,10-epithiostearamide. Elemental analysis, calculated values in parentheses was as

follows: C = 70.53 (70.19), H = 10.59 (10.94), N = 2.75 (2.10), S = 5.50 (9.59).

#### EXAMPLE 24

4-Methoxyphenyl 9,10-epithiostearate.

A. 4-Methoxyphenyl oleate — This product is prepared using 27.3 g (0.22 mole) of 4-methoxyphenol, 17.4 g (0.22 mole) of pyridine dissolved in 150 ml of benzene, and 66 g (0.22 mole) of oleoyl chloride which is added dropwise with stirring. After stirring for an additional hour the mixture is filtered, washed successively with dilute hydrochloric acid and water, and dried over anhydrous sodium sulfate. Free acid is removed by percolating the benzene solution through a column of activated alumina. The solvent is then removed by stripping under reduced pressure.

B. 4-Methoxyphenyl 9,10-epoxystearate — 31.2 g (0.18 mole) of meta chloroperbenzoic acid was dissolved in 400 ml of chloroform and added slowly to a solution containing 61 g (0.16 mole) of A and 150 ml of chloroform. After stirring for an additional hour, the excess m-chloroperbenzoic acid was destroyed using a 10% solution of sodium sulfite, after which m-chlorobenzoic acid was neutralized with Na<sub>2</sub>CO<sub>3</sub> and the solution washed with water, dried over anhydrous Na<sub>2</sub>SO<sub>4</sub> filtered and stripped.

C. 4-Methoxyphenyl 9,10-epithiostearate — 11.9 g (.16 mole) thiourea in 60 ml of water was added to 7.9 g (.08 mole) of sulfuric acid in 40 ml of water. The mixture was cooled to 5°C after which 63 g (0.16 mole) of 4-methoxyphenyl 9,10-epoxystearate which was dissolved in 150 ml of dioxane was added to the mixture with stirring over a two-hour period, the temperature being maintained at 5°C. After the addition, the mixture was heated to 40°C, the heat removed and then stirred for two hours. The mixture was neutralized with 8.5 g (.08 mole) of anhydrous sodium carbonate in 100 ml of water and warmed to 40°C. The heat was removed and the reaction continued for one hour. The mixture was extracted with 3-50 ml portions of diethyl ether, after which the ether extract was washed with water until neutral, dried over anhydrous sodium sulfate and stripped. % S 4.79 (7.61).

#### EXAMPLE 25

2-(2-Ethoxyethoxy)ethyl 9,10-epithiostearate.

This product was prepared as described in Example 24 from 19.1 g (0.25 mole) of thiourea, 12.7 g (0.13 mole) of sulfuric acid and 92.8 g (0.25 mole) of 2-(2-ethoxyethoxy)ethyl 9,10-epoxystearate. % S 6.20 (.7.43).

#### EXAMPLE 26

2-Ethoxyethyl 9,10-epithiostearate.

This product was prepared as described in Example 24 from 18.5 g (0.24 mole) of thiourea, 11.8 g (0.12 mole) of sulfuric acid and 90 g (0.24 mole) of 2-ethoxyethyl-9,10-epoxystearate. % S 5.74, (8.28).

#### EXAMPLE 27

2-Ethoxyphenyl 9,10-epithiostearate.

This product was prepared as described in Example 24 from 19.3 g (0.25 mole) of thiourea, 12.3 g (0.13 mole) of sulfuric acid, and 106 g (0.25 mole) of 2-ethoxyphenyl-9,10-epoxystearate. % S 5.1 (7.36).

## EXAMPLE 28

## 1,3-Bis(9,10-Epithiostearoyl)imidazolidine

A. N,N'-Ethylenebisoleamide — This product was prepared by adding with stirring 200 g (0.66 moles) of oleoyl chloride to 19.9 g (0.33 mole) of ethylenediamine in the presence of 52.6 g (0.66 mole) of pyridine using benzene as a solvent. After filtration employing a Buchner funnel, the filtrate was washed with dilute hydrochloric acid, followed by water, then was dried over anhydrous sodium sulfate, filtered and stripped. N,N'-ethylene bis oleamide was recrystallized twice from acetone.

B. 1,3-Dioleoylimidazolidine — 1,3-Dioleoylimidazolidine was prepared from 71.5 g (0.12 mole) of N,N'-ethylenebisoleamide and 21.8 g formaldehyde solution (36.8%) in 150 ml of acetic acid containing a catalytic amount (4 ml) of 37% hydrochloric acid. Those materials were placed in a flask and stirred by means of a magnetic stirring bar while the temperature was raised to 50°C and held at this temperature for 2 hours. Then the acetic acid, excess formaldehyde solution and hydrochloric acid were removed by distillation at reduced pressure. The product was recrystallized twice from absolute ethyl alcohol and dried in a vacuum desiccator over phosphorus pentoxide.

C. 1,3-Bis(9,10-epoxystearoyl)imidazolidine — This product was prepared as described in Example 24 from

56 g (0.10 mole) of 1,3-dioleoylimidazolidine and 37 g (.21 mole) of m-chloroperbenzoic acid.

D. 1,3-Bis(9,10-epithiostearoyl)imidazolidine — This product was prepared as described in Example 24 from 15 g (0.20 mole) of thiourea, 9.8 g (0.1 mole) of sulfuric acid and 61.8 g (0.098 mole) of 1,3-bis(9,10-epoxystearoyl)imidazolidine. % S 5.18 (9.62).

## EXAMPLE 29

10 1,3-Bis(9,10-epithiostearoyl)hexahydropyrimidine — This product was prepared as described in Example 28 from 13 g (0.17 mole) of thiourea, 8.3 g (0.085 mole) of sulfuric acid and 55 g (0.085 mole) of 1,3-bis(9,10-epoxystearoyl)hexahydropyrimidine. % S 4.29 (9.43).

## EXAMPLE 30

The compounds prepared in accordance to the procedures given in Examples 1 through 29 were evaluated 20 as base lubricants in the Shell Four-Ball Wear tests following a modified procedure of ASTM D2266-67. The resulting scar diameter on the balls after running at 600 rpm for 1 hour at 120°C and 50 Kg load were compared with the scars obtained using commercial lubricants 25 such as Aeroshell Mil-L-708 (Di-2-ethylhexyl sebacate and additive), Gulfpride, single G, MS, multiviscosity, and 100 sec. paraffin oil. The results of these tests are reported in Table I and Table IA A.

TABLE I

## ANTIWEAR LUBRICANT PROPERTIES OF FATTY ACID AMIDES

| COMPOUND                                                            | Avg. Wear Scar, mm |                  | Additive                            |
|---------------------------------------------------------------------|--------------------|------------------|-------------------------------------|
|                                                                     | without additive   | with 5% additive |                                     |
| 1. N,N-Bis(2-ethoxyethyl)oleamide                                   | 0.597              | 0.735            | N,N-Di-butyl-9,10-epithiostearamide |
| 2. N,N-Di-n-butyl-9,10-epithiostearamide                            | 0.842              | —                | none                                |
| 3. Oleoylmorpholine                                                 | 0.623              | 0.658            | "                                   |
| 4. N,N-Dimethyloleamide                                             | 0.797              | 0.987            | "                                   |
| 5. N,N-Di-n-propyloleamide                                          | 0.908              | 0.885            | "                                   |
| 6. N,N-Di-n-hexyloleamide                                           | 0.893              | 0.898            | "                                   |
| 7. N,N-Di-n-butylerucamide                                          | 0.758              | 0.798            | "                                   |
| 8. N,N-Di-n-butyl amide of Sel. hydrogenated cottonseed fatty acids | 0.798              | 0.958            | "                                   |
| 9. N,N-Bis(2-Methoxyethyl)oleamide                                  | 0.626              | 0.725            | "                                   |
| 10. N,N-Dibutyooleamide                                             | 0.710              | —                | —                                   |
| 11. N-Oleoyl-4-propyl-piperidine                                    | 0.847              | —                | —                                   |
| 12. Morpholide of sel. hydrogenated cottonseed fatty acids          | 0.642              | —                | —                                   |
| 13. N-Methyl-N-butyl-oleamide                                       | 0.607              | —                | —                                   |
| 14. N-Ethoxyethoxyethoxypropyoleamide                               | 0.503              | —                | —                                   |
| 15. N-Ethoxyethoxypropyl-oleamide                                   | 0.526              | —                | —                                   |
| 16. N-Methoxyisopropyl-oleamide                                     | 0.705              | —                | —                                   |

TABLE I—Continued

| ANTIWEAR LUBRICANT PROPERTIES OF FATTY ACID AMIDES                |                    |                                                               |          |
|-------------------------------------------------------------------|--------------------|---------------------------------------------------------------|----------|
| COMPOUND                                                          | Avg. Wear Scar, mm |                                                               |          |
|                                                                   | without additive   | with 5% additive                                              | Additive |
| 17. N-Methoxyethyloleamide                                        | 0.420              | —                                                             | —        |
| 18. 102 sec Paraffin Oil                                          | 0.902              | N-Methoxyethyloleamide                                        |          |
| 19. D.O.S.                                                        | 0.906              | “                                                             |          |
| 20. N,N-Dibutyl-9(10)-carbobutoxyoctadecanamide                   | 0.610              | —                                                             |          |
| 21. 102 sec Paraffin Oil                                          | 0.818              | N,N-Dibutyl-9(10)-carbobutoxyoctadecanamide                   |          |
| 22. D.O.S.                                                        | 0.945              | “                                                             |          |
| 23. N-[9(10)mercaptop-(9)10-dibutylphosphatostearoyl]morpholine   | 0.615              | —                                                             |          |
| 24. 102 sec Paraffin Oil                                          | 0.552              | N-[9(10)mercaptop-(9)10-dibutylphosphatostearoyl]morpholine   |          |
| 25. D.O.S.                                                        | 0.535              | “                                                             |          |
| 26. N,N-Dibutyl-[9(10)-hydroxy-(9)10-di-butylphosphato]stearamide | 0.498              | —                                                             |          |
| 27. 102 sec Paraffin Oil                                          | 0.498              | N,N-Dibutyl-[9(10)-hydroxy-(9)10-di-butylphosphato]stearamide |          |
| 28. D.O.S.                                                        | 0.498              |                                                               |          |
| 29. N,N-Dibutyl-9(10)-[dibutylphosphono]stearamide                | 0.530              | —                                                             |          |
| 30. N-Ethoxyethoxyethoxypropyl-9,10-epithiostearamide             | 0.707              | —                                                             |          |
| 31. N-Ethoxyethoxyethoxypropyl-9(10)mercaptopstearamide           | 0.690              | —                                                             |          |
| 32. N-(9,10-12,13-diepithiostearoyl)morpholine                    | 0.665              | —                                                             |          |
| 33. Bis(2-ethylhexyl)sebacate                                     | 0.872              | —                                                             | —        |
| 34. 100 sec Paraffin Oil                                          | 0.803              | —                                                             | —        |
| 35. Aero Shell (Mil-7808)                                         | 0.587              |                                                               |          |
| 36. Gulf Pride, Single G, MS, multiviscosity                      | 0.447              |                                                               |          |
| 37. 100 sec Paraffin Oil                                          | 0.813              | N,N-Dibutyl-9,10-12,13-Diepithiostearamide                    |          |
| 38. Bis(2-ethylhexyl)sebacate                                     | 0.836              | “                                                             |          |
| 39. 100 sec Paraffin Oil                                          | 0.723              | N-9,10-epithiostearoyl morpholine                             |          |
| 40. Bis(2-ethylhexyl)sebacate                                     | 0.915              | “                                                             |          |
| 41. 100 sec Paraffin Oil                                          | 0.917              | N,N-Dibutyl-9,10-dichlorostearamide                           |          |
| 42. Bis(2-ethylhexyl)sebacate                                     | 0.848              | “                                                             |          |

TABLE IA

It can be seen from the data presented that the N-alkoxyalkyl and N,N-di(alkoxyalkyl)oleamides, without the assistance of additives, exhibited wear characteristics (i.e., low scar diameters) comparable to the commercial controls Aeroshell and Gulfpride which do contain additives to improve performance. N,N-dibutyl-[9(10)-hydroxy-(9)10-dibutylphosphato]-stearamide and N-[9(10)mercapto-(9)10-dibutylphosphatostearoyl]morpholine not only exhibit low wear characteristics in themselves but also impart as additives such characteristics to paraffin oil and DOS base lubricants. A large number of these, particularly the esters and ester amides such as PC-O-7857, 7858, 7859, 7887, 7953, 7954, 7955, 7956, 7958, and 7959, although poor in wear characteristics as base oils, are very effective anti-wear additives for either paraffinic or diester base oils, in some instances both.

## EXAMPLE 31

The various amides were evaluated as extreme pressure lubricants or additives in a Shell 4-ball extreme pressure tester at 1,440 PPM following ASTM Procedure D 2596-67T. Loads were increased in increments of 20 Kg to weld point and the test ran for one minute or to weld whichever occurred first. Commercial hypoid fluid SAE No. 90 was employed as the control E.P. lubricant. The performance of the amides tested is given in Tables II, III, and IV.

TABLE II

| EXTREME PRESSURE TESTS (ASTM D2506-67T) |                                                             |                                |                                  |
|-----------------------------------------|-------------------------------------------------------------|--------------------------------|----------------------------------|
|                                         | COMPOUND                                                    | Weld Point<br>(No<br>additive) | Weld Point<br>(with 5%<br>No. 2) |
| 1                                       | N,N-Bis(2-ethoxyethyl)oleamide                              | 120                            | 170                              |
| 2                                       | N,N-Di-n-butyl-9,10-epithiostearamide                       | 300                            | —                                |
| 3                                       | Oleylmorpholine                                             | 120                            | 150                              |
| 4                                       | N,N-Dimethyoieamide                                         | 120                            | 140                              |
| 5                                       | N,N-Di-n-propyloleamide                                     | 120                            | 150                              |
| 6                                       | N,N-Di-n-hexyloleamide                                      | 120                            | 180                              |
| 7                                       | N,N-Di-n-butylceramide                                      | 120                            | 200                              |
| 8                                       | N,N-Di-n-butyl amide of hydrogenated cottonseed fatty acids | 120                            | 170                              |
| 9                                       | N,N-Bis(2-Methoxyethyl)oleamide                             | 120                            | 160                              |
| 10                                      | N-Methyl-N-butylolamide                                     | 100                            | —                                |
| 11                                      | N,N-Dibutyl-9,10-epithiostearamide                          | 300                            | —                                |
| 12                                      | N,N-Dibutyl-9,10-12,13-diepithiostearamide                  | 440                            | —                                |
| 13                                      | N-Ethoxyethoxyethoxypropyoleamide                           | 120                            | —                                |
| 14                                      | N-Ethoxyethoxypropyoleamide                                 | 120                            | —                                |
| 15                                      | N-Methoxyisopropylolamide                                   | 100                            | —                                |
| 16                                      | N-Methoxyethyloleamide                                      | 100                            | —                                |
| 17                                      | N-9,10-epithiostearoylmorpholine                            | 380                            | —                                |

TABLE II-Continued

## EXTREME PRESSURE TESTS (ASTM D2506-67T)

|     | COMPOUND                           | Weld Point<br>(No<br>additive) | Weld Point<br>(with 5%<br>No. 2) |
|-----|------------------------------------|--------------------------------|----------------------------------|
| 18. | Bis(2-ethylhexyl)sebacate          | 120                            | —                                |
| 19. | 100 sec Paraffin Oil               | 100                            | —                                |
| 20. | SAE No. 90 Commercial hypoid fluid | 280                            | —                                |

TABLE III

## EVALUATION OF N,N-DIBUTYL-9,10-12,13-DI-EPITHIOSTEARAMIDE AS AN ADDITIVE AND AS A BASE OIL IN EXTREME PRESSURE TESTS. (ASTM D2596-67T)

| BASE OIL                   | % ADDITIVE | LOAD, Kg                | WEAR SCAR mm |
|----------------------------|------------|-------------------------|--------------|
| 100 sec Paraffin Oil       | (5%)       | 140                     | 1.90         |
| "                          | "          | 200                     | 2.35         |
| "                          | "          | 220                     | 2.75         |
| "                          | "          | 240                     | Weld—5 sec.  |
| Bis(2-ethylhexyl)-sebacate | (5%)       | 120                     | 1.51         |
| "                          | "          | 180                     | 1.59         |
| "                          | "          | 190 (T.S.) <sup>a</sup> | 2.47         |
| "                          | "          | 200                     | Weld—4 sec.  |
| "                          | (10%)      | 240                     | 2.88         |
| "                          | "          | 260                     | 3.55         |
| "                          | "          | 270                     | Weld—10 sec. |

<sup>a</sup>Incipient seizure

## EXTREME PRESSURE TESTS ON N-ETHOXYETHOXYETHOXYPROPYL-9,10-EPITHIOSTEARAMIDE (PC-O-No. 7682)

| BASE OIL | ADDITIVE | APPLIED LOAD | AVE. SCAR mm |
|----------|----------|--------------|--------------|
| 7682     | None     | 120          | 1.05         |
| "        | "        | 160          | 1.75         |
| "        | "        | 240          | 2.35         |
| "        | "        | 300          | 2.19         |
| "        | "        | 340          | 2.55         |
| "        | "        | 360          | 2.62         |
| "        | "        | 380          | weld         |

## EVALUATION OF ETHOXYETHOXYETHOXYPROPYL PENTACHLOROSTEARAMIDE (PC-O-7857) AS AN ADDITIVE IN EXTREME PRESSURE TESTS

| Base Oil         | Additive<br>5% | Load, Kg | Wear Scar, mm |
|------------------|----------------|----------|---------------|
| D.O.S.           | PC-O-7857      | 160      | 3.38          |
| "                | "              | 180      | 3.06          |
| "                | "              | 200      | 2.93          |
| "                | "              | 220      | 3.05          |
| "                | "              | 230      | Weld—17 sec.  |
| 102 Paraffin Oil | PC-O-7857      | 140      | 2.10          |
| "                | "              | 170      | 2.91          |
| "                | "              | 180      | Weld—22 sec.  |

TABLE III-Continued

EVALUATION OF  
N-METHYL-N-[2-(9,10-EPITHIOSTEARYLOXY)ETHYL]-9,10-  
EPITHIOSTEARAMIDE (PC-O-7858) AS AN ADDITIVE AND A  
BASE OIL IN EXTREME PRESSURE TESTS

| Base Oil             | Additive  | 5%  | Load, Kg       | Wear Scar, mm |
|----------------------|-----------|-----|----------------|---------------|
| PC-O-7858            | none      | 120 | 0.833          |               |
| "                    | "         | 200 | 1.71           |               |
| "                    | "         | 260 | 2.08           |               |
| "                    | "         | 300 | 1.88           |               |
| "                    | "         | 360 | 2.37           |               |
| "                    | "         | 420 | 2.42           |               |
| "                    | "         | 460 | 2.57           |               |
| "                    | "         | 480 | 3.15           |               |
| "                    | "         | 490 | Weld — 3 sec.  |               |
| D.O.S.               | PC-O-7858 | 120 | 2.55           |               |
| "                    | "         | 140 | 2.95           |               |
| "                    | "         | 200 | 3.43           |               |
| "                    | "         | 210 | 3.52           |               |
| "                    | "         | 220 | Weld — 20 sec. |               |
| S105 Topaz Oil       | PC-O-7858 | 120 | 2.65           |               |
| "                    | "         | 160 | 3.28           |               |
| "                    | "         | 180 | 3.32           |               |
| "                    | "         | 190 | Weld — 17 sec. |               |
| S105 Topaz Oil       | none      | 120 | Weld — 15 sec. |               |
| 102 sec Paraffin Oil | 7682 (5%) | 120 | 2.28           |               |
| "                    | "         | 140 | 2.46           |               |
| "                    | "         | 150 | weld           |               |
| D.O.S.               | 7682 (5%) | 120 | 2.23           |               |
| "                    | "         | 140 | 2.44           |               |
| "                    | "         | 150 | weld           |               |

EXTREME PRESSURE TESTS ON  
N-ETHOXYETHOXYETHOXYPROPYL-9(10)-MERCAPTO-

| BASE OIL             | ADDITIVE  | APPLIED LOAD, Kg | AVE. SCAR, mm     |
|----------------------|-----------|------------------|-------------------|
| 7683                 | None      | 200              | 1.54              |
| "                    | "         | 300              | 2.26              |
| "                    | "         | 400              | 2.25              |
| "                    | "         | 450              | 2.15              |
| "                    | "         | 500              | 2.15 <sup>1</sup> |
| 102 sec Paraffin Oil | 7683 (5%) | 120              | 1.97              |
| "                    | "         | 140              | 2.35              |
| "                    | "         | 150              | 2.54              |
| "                    | "         | 160              | weld              |
| D.O.S.               | 7683 (5%) | 120              | 1.68              |
| "                    | "         | 140              | 2.18              |
| "                    | "         | 160              | 2.59              |
| "                    | "         | 170              | 2.72              |
| "                    | "         | 180              | weld              |

<sup>1</sup> Test stopped because of extreme decomposition. Did not weld.

EXTREME PRESSURE TESTS ON  
N-(9,10-12,13-DIEPITHIOSTEARYOL)MORPHOLINE (PC-O-No.  
7684)

| BASE OIL                   | ADDITIVE  | APPLIED LOAD, Kg | AVG. SCAR, mm     |
|----------------------------|-----------|------------------|-------------------|
| 7684                       | None      | 200              | 2.21              |
| "                          | "         | 260              | 2.38              |
| "                          | "         | 340              | 2.43              |
| "                          | "         | 400              | 2.75              |
| "                          | "         | 460              | 2.90              |
| "                          | "         | 500              | 2.98 <sup>1</sup> |
| 102 sec Paraffin Oil       | 7684 (5%) | 100              | 2.23              |
| "                          | "         | 120              | 2.61              |
| "                          | "         | 130              | 2.74              |
| "                          | "         | 140              | weld              |
| D.O.S.                     | 7684 (5%) | 120              | 2.54              |
| "                          | "         | 140              | 2.58              |
| "                          | "         | 150              | weld              |
| N-methoxyethyl<br>oleamide | 7684 (5%) | 140              | 2.53              |

TABLE III-Continued

EXTREME PRESSURE TESTS ON  
N-(9,10-12,13-DIEPITHIOSTEARYOL)MORPHOLINE  
(PC-O-No. 7684)

| 5 | BASE OIL | ADDITIVE | APPLIED LOAD, Kg | AVG. SCAR, mm |
|---|----------|----------|------------------|---------------|
| " | "        | "        | 160              | 2.77          |
| " | "        | "        | 170              | weld          |

<sup>1</sup> Test stopped because of extreme decomposition. Did not weld.

EXTREME PRESSURE TESTS ON  
N,N-DIBUTYL-9(10)-(DIBUTYLPHOSPHONO)STEARAMIDE  
(PC-O-No. 7685)

| 10 | BASE OIL | ADDITIVE | APPLIED LOAD, Kg | AVE. SCAR, mm |
|----|----------|----------|------------------|---------------|
| "  | "        | "        | 120              | 3.05          |
| "  | "        | "        | 140              | 4.50          |
| "  | "        | "        | 150              | weld          |

EXTREME PRESSURE TESTS ON  
N,N-DIBUTYL-[9(10)-HYDROXY-9(10)-DIBUTYLPHOS-  
PHATO]STEARAMIDE (PC-O-No. 7686)

| 20 | 7686 | None | 200 | 0.887 |
|----|------|------|-----|-------|
| "  | "    | "    | 300 | 2.78  |
| "  | "    | "    | 340 | 4.32  |
| "  | "    | "    | 350 | 4.50  |
| "  | "    | "    | 360 | weld  |

| 25 | 100 sec<br>Paraffin Oil | 7686 (5%) | 120 | 2.28 |
|----|-------------------------|-----------|-----|------|
| "  | "                       | "         | 140 | 2.80 |
| "  | "                       | "         | 150 | 3.01 |
| "  | "                       | "         | 160 | weld |
| 30 | D.O.S.                  | 7686 (5%) | 120 | 1.95 |
| "  | "                       | "         | 140 | 2.85 |
| "  | "                       | "         | 150 | 3.03 |
| "  | "                       | "         | 160 | weld |

EXTREME PRESSURE TESTS ON  
N-[9(10)-MERCAPTO-9(10)-DIBUTYLPHOSPHATOS-  
TEAROYL]MORPHOLINE (PC-O-No. 7687)

| 35 | BASE OIL | ADDITIVE | APPLIED LOAD, Kg | AVE. SCAR, mm     |
|----|----------|----------|------------------|-------------------|
| "  | "        | "        | 120              | 0.608             |
| "  | "        | "        | 160              | 1.35              |
| "  | "        | "        | 200              | 1.40              |
| "  | "        | "        | 240              | 1.70              |
| "  | "        | "        | 280              | 3.36 <sup>1</sup> |

EXTREME PRESSURE TESTS ON  
N,N-DIBUTYL-9(10)-CARBOBUTYXYOCATDECANAMIDE  
(PC-O-No. 7688)

| 40 | 7688 | None | 80  | 1.92 |
|----|------|------|-----|------|
| "  | "    | "    | 90  | 2.18 |
| "  | "    | "    | 100 | 2.45 |
| "  | "    | "    | 120 | weld |

EVALUATION OF  
N-[2-(9,10-EPITHIOSTEARYLOXY)ETHYL]-9,10-EPITHIOS-  
TEARAMIDE (PC-O-7859) AS AN ADDITIVE AND A BASE OIL IN  
EXTREME PRESSURE TESTS

| 50 | Base Oil         | Additive  | Load, Kg | Wear Scar, mm  |
|----|------------------|-----------|----------|----------------|
| "  | PC-O-7859        | none      | 120      | 1.17           |
| "  | "                | "         | 200      | 1.62           |
| "  | "                | "         | 300      | 2.05           |
| "  | "                | "         | 400      | 2.37           |
| "  | "                | "         | 460      | 2.48           |
| "  | "                | "         | 500      | 3.22           |
| "  | "                | "         | 520      | 3.47           |
| "  | "                | "         | 530      | Weld — 10 sec. |
| 60 | D.O.S.           | PC-O-7859 | 120      | 1.69           |
| "  | "                | "         | 140      | 1.82           |
| "  | "                | "         | 150      | 2.18           |
| "  | "                | "         | 160      | Weld — 60 sec. |
| 65 | 102 Paraffin Oil | PC-O-7859 | 120      | 1.80           |
| "  | "                | "         | 160      | 2.18           |
| "  | "                | "         | 180      | 2.43           |
| "  | "                | "         | 190      | 2.51           |
| "  | "                | "         | 200      | Weld — 52 sec. |

TABLE III-Continued

| EVALUATION OF<br>ETHOXYETHOXYETHOXYPROPYL-9,10-12,13-DIEPITHIOS-<br>TEARAMIDE (PC-0-7861) AS AN ADDITIVE AND A BASE OIL IN<br>EXTREME PRESSURE TESTS |           |          |               |    |
|------------------------------------------------------------------------------------------------------------------------------------------------------|-----------|----------|---------------|----|
| Base Oil                                                                                                                                             | Additive  | Load, Kg | Wear Scar, mm |    |
| PC-0-7861                                                                                                                                            | none      | 120      | 1.01          | 5  |
| "                                                                                                                                                    | "         | 200      | 2.22          |    |
| "                                                                                                                                                    | "         | 300      | 2.02          |    |
| "                                                                                                                                                    | "         | 400      | 2.19          |    |
| "                                                                                                                                                    | "         | 500      | 2.43          |    |
| "                                                                                                                                                    | "         | 600"     | 2.48          |    |
| D.O.S.                                                                                                                                               | PC-0-7861 | 120      | 1.93          | 10 |
| "                                                                                                                                                    | "         | 160      | 2.48          |    |
| "                                                                                                                                                    | "         | 170      | 2.78          |    |
| "                                                                                                                                                    | "         | 180      | Weld — 3 sec. |    |
| 102 Paraffin Oil                                                                                                                                     | PC-0-7861 | 120      | 1.37          | 15 |
| "                                                                                                                                                    | "         | 160      | 2.31          |    |
| "                                                                                                                                                    | "         | 180      | 1.59          |    |
| "                                                                                                                                                    | "         | 190      | 2.26          |    |
| "                                                                                                                                                    | "         | 200      | Weld — 5 sec. |    |

"No weld point; very little decomposition.

| EVALUATION OF<br>N-METHYL-N-PHENYL-9,10-EPITHIOSTEARAMIDE<br>(PC-0-7871) AS AN ADDITIVE AND AS A BASE OIL IN<br>EXTREME PRESSURE TESTS |           |          |                |    |
|----------------------------------------------------------------------------------------------------------------------------------------|-----------|----------|----------------|----|
| Base Oil                                                                                                                               | Additive  | Load, Kg | Wear Scar, mm  |    |
| PC-0-7871                                                                                                                              | none      | 120      | 1.35           | 25 |
| "                                                                                                                                      | "         | 140      | 1.93           |    |
| "                                                                                                                                      | "         | 180      | 1.87           |    |
| "                                                                                                                                      | "         | 220      | 1.89           |    |
| "                                                                                                                                      | "         | 300      | 2.74           |    |
| "                                                                                                                                      | "         | 400      | 2.40           |    |
| "                                                                                                                                      | "         | 420      | 2.95           | 30 |
| "                                                                                                                                      | "         | 440      | Weld — 30 sec. |    |
| D.O.S.                                                                                                                                 | PC-0-7871 | 120      | 2.35           |    |
| "                                                                                                                                      | "         | 140      | 3.17           |    |
| "                                                                                                                                      | "         | 150      | 3.23           |    |
| "                                                                                                                                      | "         | 160      | Weld — 10 sec. |    |
| 102 Paraffin Oil                                                                                                                       | PC-0-7871 | 120      | 2.53           | 35 |
| "                                                                                                                                      | "         | 130      | 2.62           |    |
| "                                                                                                                                      | "         | 140      | Weld — 20 sec. |    |

| EVALUATION OF<br>1,3-BIS(9,10-EPITHIOSTEAROXYLOXY)PROPANE (PC-0-7863)<br>AS AN ADDITIVE AND A BASE OIL IN EXTREME PRESSURE<br>TESTS |           |          |                |    |
|-------------------------------------------------------------------------------------------------------------------------------------|-----------|----------|----------------|----|
| Base Oil                                                                                                                            | Additive  | Load, kg | Wear Scar, mm  |    |
| PC-0-7863                                                                                                                           | none      | 120      | 0.90           | 50 |
| "                                                                                                                                   | "         | 200      | 1.21           |    |
| "                                                                                                                                   | "         | 300      | 2.23"          |    |
| "                                                                                                                                   | "         | 340      | 3.42"          |    |
| "                                                                                                                                   | "         | 360      | 2.85"          |    |
| "                                                                                                                                   | "         | 380      | 3.17"          |    |
| "                                                                                                                                   | "         | 390      | 3.47"          | 55 |
| "                                                                                                                                   | "         | 400      | Weld — 2 sec.  |    |
| D.O.S.                                                                                                                              | PC-0-7863 | 120      | 2.49           |    |
| "                                                                                                                                   | "         | 140      | 2.65           |    |
| "                                                                                                                                   | "         | 160      | 2.78           |    |
| "                                                                                                                                   | "         | 180      | 3.18           |    |
| "                                                                                                                                   | "         | 190      | Weld — 8 sec.  | 60 |
| S105 Topaz Oil                                                                                                                      | PC-0-7863 | 120      | 2.37           |    |
| "                                                                                                                                   | "         | 140      | 2.67           |    |
| "                                                                                                                                   | "         | 150      | 2.72           |    |
| "                                                                                                                                   | "         | 170      | Weld — 10 sec. | 65 |
| S105 Topaz Oil                                                                                                                      | none      | 120      | Weld — 15 sec. |    |

"Some Corrosion

TABLE III-Continued

| EVALUATION OF<br>1,3-DI(9,10-EPITHIOSTEAROYL)HEXAHYDROPRIMIDINE<br>(PC-0-7887) AS AN ADDITIVE AND A BASE OIL IN EXTREME<br>PRESSURE TESTS |           |          |                |    |
|-------------------------------------------------------------------------------------------------------------------------------------------|-----------|----------|----------------|----|
| Base Oil                                                                                                                                  | Additive  | Load, Kg | Wear Scar, mm  |    |
| PC-0-7887                                                                                                                                 | none      | 120      | 0.782          | 5  |
| "                                                                                                                                         | "         | 200      | 1.78           |    |
| "                                                                                                                                         | "         | 300      | 2.92           |    |
| "                                                                                                                                         | "         | 310      | 3.00           |    |
| "                                                                                                                                         | "         | 320      | Weld — 30 sec. |    |
| D.O.S.                                                                                                                                    | PC-0-7887 | 120      | 2.30           |    |
| "                                                                                                                                         | "         | 140      | 2.48           | 10 |
| "                                                                                                                                         | "         | 160      | 2.74           |    |
| "                                                                                                                                         | "         | 170      | 2.89           |    |
| "                                                                                                                                         | "         | 180      | Weld — 10 sec. |    |
| S105 Topaz Oil                                                                                                                            | PC-0-7887 | 120      | 2.81           | 15 |
| "                                                                                                                                         | "         | 130      | 2.94           |    |
| "                                                                                                                                         | "         | 140      | Weld — 15 sec. |    |
| S105 Topaz Oil                                                                                                                            | none      | 120      | Weld — 15 sec. |    |

EVALUATION OF 2-ETHOXYETHYL 9,10-EPITHIOSTEARATE  
(PC-0-7953) AS AN ADDITIVE IN EXTREME PRESSURE TESTS

Base Oil Additive, 5% Load, kg Wear Scar, mm

|    |                |           |     |               |
|----|----------------|-----------|-----|---------------|
| 25 | D.O.S.         | PC-0-7953 | 120 | 1.13          |
|    | "              | "         | 160 | 2.65          |
|    | "              | "         | 200 | 2.97          |
|    | "              | "         | 240 | 2.99          |
|    | "              | "         | 250 | Weld — 7 sec. |
| 30 | Topaz S105 Oil | PC-0-7953 | 120 | 2.47          |
|    | "              | "         | 150 | 2.68          |
|    | "              | "         | 160 | Weld — 4 sec. |

EVALUATION OF 2-(2-ETHOXYETHOXY)ETHYL  
9,10-EPITHIOSTEARATE (PC-0-7954) AS AN ADDITIVE IN  
EXTREME PRESSURE TESTS

Base Oil Additive, 5% Load, kg Wear Scar, mm

|    |                |           |     |                |
|----|----------------|-----------|-----|----------------|
| 35 | D.O.S.         | PC-0-7954 | 120 | 0.885          |
|    | "              | "         | 160 | 2.72           |
|    | "              | "         | 170 | Weld — 9 sec.  |
| 40 | Topaz S105 Oil | PC-0-7954 | 120 | 2.45           |
|    | "              | "         | 140 | 3.17           |
|    | "              | "         | 150 | Weld — 10 sec. |

EVALUATION OF 2-ETHOXYPHENYL 9,10-EPITHIOSTEARATE  
(PC-0-7955) AS AN ADDITIVE IN EXTREME PRESSURE TESTS

Base Oil Additive, 5% Load, kg Wear Scar, mm

|    |                |           |     |               |
|----|----------------|-----------|-----|---------------|
| 45 | D.O.S.         | PC-0-7955 | 120 | 0.863         |
|    | "              | "         | 160 | 2.62          |
|    | "              | "         | 170 | Weld — 7 sec. |
| 50 | Topaz S105 Oil | PC-0-7955 | 120 | 2.24          |
|    | "              | "         | 140 | 2.51          |
|    | "              | "         | 150 | 2.75          |
|    | "              | "         | 160 | Weld — 6 sec. |

EVALUATION OF 4-METHOXYPHENYL  
9,10-EPITHIOSTEARATE (PC-0-7956) AS AN ADDITIVE IN  
EXTREME PRESSURE TESTS

Base Oil Additive, 5% Load, kg Wear Scar, mm

|    |                |           |     |               |
|----|----------------|-----------|-----|---------------|
| 55 | D.O.S.         | PC-0-7956 | 120 | 0.963         |
|    | "              | "         | 180 | 1.04          |
|    | "              | "         | 190 | 3.35          |
|    | "              | "         | 200 | Weld — 6 sec. |
| 60 | Topaz S105 Oil | PC-0-7956 | 120 | 2.38          |
|    | "              | "         | 140 | 2.37          |
|    | "              | "         | 180 | 2.95          |
|    | "              | "         | 200 | 3.78          |
|    | "              | "         | 210 | Weld — 4 sec. |

TABLE III-Continued

EVALUATION OF  
1,3-BIS-(9,10-EPITHIOSTEAROYL)-IMIDAZOLIDINE  
(PC-0-7957) AS AN ADDITIVE IN EXTREME PRESSURE TESTS

| Base Oil       | Additive, 5% | Load, kg | Wear Scar, mm |    |
|----------------|--------------|----------|---------------|----|
| D.O.S.         | PC-0-7957    | 120      | 1.42          |    |
|                | "            | 150      | 0.897         |    |
|                | "            | 180      | 1.23          |    |
|                | "            | 200      | 3.00          |    |
|                | "            | 240      | 3.14          | 10 |
|                | "            | 260      | Weld — 8 sec. |    |
| Topaz S105 Oil | PC-0-7957    | 120      | 0.855         |    |
|                | "            | 160      | 1.01          |    |
|                | "            | 200      | 1.09          |    |
|                | "            | 260      | 1.17          |    |
|                | "            | 280      | 2.68          | 15 |
|                | "            | 290      | Weld — 8 sec. |    |

EVALUATION OF EPITHIOATED SOYBEAN OIL (PC-0-7958) AS  
AN ADDITIVE AND AS A BASE OIL IN EXTREME PRESSURE  
TESTS

| Base Oil       | Additive, 5% | Load, kg         | Wear Scar, mm |    |
|----------------|--------------|------------------|---------------|----|
| PC-0-7958      | none         | 120              | 0.775         |    |
|                | "            | 200              | 1.49          |    |
|                | "            | 260              | 1.63          |    |
|                | "            | 320              | 1.89          |    |
|                | "            | 400              | 2.10          |    |
|                | "            | 500 <sup>a</sup> | 2.15          | 25 |
| D.O.S.         | PC-0-7958    | 120              | 1.53          |    |
|                | "            | 150              | 1.03          |    |
|                | "            | 200              | 1.15          |    |
|                | "            | 260              | 1.77          |    |
|                | "            | 280              | 2.70          |    |
|                | "            | 290              | 2.78          | 30 |
| Topaz S105 Oil | PC-0-7958    | 120              | 2.23          |    |
|                | "            | 150              | 2.60          |    |
|                | "            | 180              | 2.67          |    |
|                | "            | 200              | Weld — 9 sec. | 35 |

<sup>a</sup>Test stopped because of harsh fumes and decomposition.EVALUATION OF 9,10-EPITHIOSTEARYL  
9,10-EPITHIOSTEARATE (PC-0-7959) AS AN ADDITIVE AND AS  
A BASE OIL IN EXTREME PRESSURE TESTS

| Base Oil       | Additive, 5% | Load, kg | Wear Scar, mm |    |
|----------------|--------------|----------|---------------|----|
| PC-0-7959      | none         | 120      | 1.40          |    |
|                | "            | 160      | 1.74          |    |
|                | "            | 200      | 1.75          |    |
|                | "            | 300      | 3.77          |    |
|                | "            | 310      | Weld — 9 sec. | 45 |
|                |              |          |               |    |
| D.O.S.         | PC-0-7959    | 120      | 1.90          |    |
|                | "            | 150      | 1.99          |    |
|                | "            | 200      | 2.38          |    |
|                | "            | 240      | 2.75          |    |
|                | "            | 290      | 2.89          |    |
|                | "            | 300      | Weld — 3 sec. |    |
| Topaz S105 Oil | PC-0-7959    | 120      | 1.87          |    |
|                | "            | 150      | 2.36          |    |
|                | "            | 200      | 2.95          |    |
|                | "            | 240      | 3.18          |    |
|                | "            | 280      | 3.85          |    |
|                | "            | 290      | Weld — 8 sec. |    |

EVALUATION OF 9,10-EPITHIOSTEARYL  
PENTACHLOROSTEARATE (PC-0-7960) AS AN ADDITIVE IN  
EXTREME PRESSURE TESTS

| Base Oil       | Additive, 5% | Load, kg | Wear Scar, mm |  |
|----------------|--------------|----------|---------------|--|
| D.O.S.         | PC-0-7960    | 120      | 1.87          |  |
|                | "            | 150      | 1.78          |  |
|                | "            | 200      | 3.40          |  |
|                | "            | 210      | Weld — 8 sec. |  |
|                |              |          |               |  |
|                |              |          |               |  |
| Topaz S105 Oil | PC-0-7960    | 120      | 0.993         |  |
|                | "            | 150      | 1.16          |  |
|                | "            | 200      | 1.39          |  |
|                | "            | 220      | 2.67          |  |
|                | "            | 230      | Weld — 4 sec. |  |

TABLE III-Continued

EVALUATION OF 9,10-EPITHIOSTEAROYL TERMINATED  
SEBACIC ACID—1,3-PROPANEDIOL POLYESTER (PC-0-7961)  
AS AN ADDITIVE IN EXTREME PRESSURE TESTS

| Base Oil       | Additive, 5% | Load, kg | Wear Scar, mm |  |
|----------------|--------------|----------|---------------|--|
| D.O.S.         | PC-0-7961    | 120      | 2.41          |  |
|                | "            | 150      | 3.00          |  |
|                | "            | 180      | 3.98          |  |
|                | "            | 200      | 3.86          |  |
|                | "            | 210      | Weld — 7 sec. |  |
|                |              |          |               |  |
| Topaz S105 Oil | PC-0-7961    | 120      | 2.40          |  |
|                | "            | 160      | 2.52          |  |
|                | "            | 180      | 3.01          |  |
|                | "            | 190      | Weld — 7 sec. |  |
|                |              |          |               |  |

TABLE IV

EVALUATION OF N-9,10-EPITHIOSTEAROYL MORPHOLINE  
AS AN ADDITIVE AND AS A BASE OIL IN EXTREME  
PRESSURE TESTS (ASTM D 2596-67T)

| BASE OIL                              | % ADDITIVE | LOAD Kg | WEAR SCAR mm  |
|---------------------------------------|------------|---------|---------------|
| 100 sec Paraffin Oil                  | (5%)       | 120     | 2.00          |
| "                                     | "          | 140     | 2.80          |
| "                                     | "          | 160     | 3.25          |
| "                                     | "          | 180     | weld, 10 sec. |
| Bis(2-ethylhexyl)<br>sebacate         | (5%)       | 80      | 1.57          |
|                                       | "          | 120     | 2.03          |
|                                       | "          | 140     | 2.41          |
|                                       | "          | 160     | 2.94          |
|                                       | "          | 180     | 3.00          |
|                                       | "          | 200     | weld, 5 sec.  |
| N-9,10-Epithio-<br>stearyl morpholine | None       | 120     | 0.70          |
|                                       | "          | 200     | 2.13          |
|                                       | "          | 240     | 2.43          |
|                                       | "          | 300     | 2.68          |
|                                       | "          | 380     | weld, 50 sec. |

We claim:

1. A composition of matter useful as a base lubricant with low wear characteristics consisting of a paraffin base oil and an anti-wear additive selected from the group consisting of N-methyl-N-[2-(9,10-epithiostearyl)-ethyl]-9,10-epithiostearamide, N-[2-(9,10-epithiostearyl)-ethyl]-9,10-epithiostearamide, 1,3-di(9,10-epithiostearyl)hexahydro-pyrimidine, 2-ethoxyethyl 9,10-epithiosteарате, 2-(2-ethoxyethoxy)ethyl 9,10-epithiosteарате, 1,3-bis(9,10-epithiostearyl)imidazolidine and epithioated soybean oil.
2. The composition of claim 1 wherein the anti-wear additive is N-methyl-N-[2-(9,10-epithiostearyl)-ethyl]-9,10-epithiostearamide.
3. The composition of claim 1 wherein the anti-wear additive is N-[2-(9,10-epithiostearyl)-ethyl]-9,10-epithiostearamide.
4. The composition of claim 1 wherein the anti-wear additive is 1,3-di(9,10-epithiostearyl)hexahydro-pyrimidine.
5. The composition of claim 1 wherein the anti-wear additive is 2-ethoxyethyl 9,10-epithiosteарате.

6. The composition of claim 1 wherein the anti-wear additive is 2-(2-ethoxyethoxy)ethyl 9,10-epithiostearate.

7. The composition of claim 1 wherein the anti-wear additive is epithioated soybean oil.

8. The composition of claim 1 wherein the anti-wear additive is 1,3-bis(9,10-epithiostearoyl)imidazolidine.

9. A composition of matter useful as a base lubricant with low wear characteristics consisting of a diester base oil and an anti-wear additive selected from the group consisting of N-[2-(9,10-epithiostearoyloxy)ethyl]-9,10-epithiostearamide, 2-ethoxyethyl 9,10-epithiostearate, 2-(2-ethoxyethoxy)ethyl 9,10-epithiostearate, 2-ethoxyphenyl 9,10-epithiostearate, and 9,10-epithiostearyl 9,10-epithiostearate.

10. The composition of claim 9 wherein the anti-wear additive is N-[2-(9,10-epithiostearoyloxy)ethyl]-9,10-epithiostearamide.

11. The composition of claim 9 wherein the anti-wear additive is 2-ethoxyethyl 9,10-epithiostearate.

12. The composition of claim 9 wherein the anti-wear additive is 2-(2-ethoxyethoxy)ethyl 9,10-epithiostearate.

13. The composition of claim 9 wherein the anti-wear additive is 2-ethoxyphenyl 9,10-epithiostearate.

14. The composition of claim 9 wherein the anti-wear additive is 9,10-epithiostearyl 9,10-epithiostearate.

15. An extreme pressure lubricant composition wherein the base lubricant is a paraffin base oil and the extreme pressure additive is selected from the group consisting of N-methyl-N-[2-(9,10-epithiostearoyloxy)ethyl]-9,10-epithiostearamide, N-[2-(9,10-epithiostearoyloxy)ethyl]-9,10-epithiostearamide, 1,3-bis(9,10-epithiostearoyloxy)propane, 2-ethoxyethyl 9,10-epithiostearate, 2-(2-ethoxyethoxy)ethyl 9,10-epithiostearate, 2-ethoxyphenyl 9,10-epithiostearate, 4-methoxyphenyl 9,10-epithiostearate, 1,3-bis(9,10-epithiostearoyl)-imidazolidine, epithioated soybean oil, 9,10-epithiostearyl 9,10-epithiostearate, 9,10-epithiostearyl pentachlorostearate, and 9,10-epithiostearoyl terminated sebacic acid-1,3-propanediol polyester.

16. The composition of claim 15 wherein the extreme pressure additive is N-methyl-N-[2-(9,10-epithiostearoyloxy)ethyl]-9,10-epithiostearamide.

17. The composition of claim 15 wherein the extreme pressure additive is N-[2-(9,10-epithiostearoyloxy)ethyl]-9,10-epithiostearamide.

18. The composition of claim 15 wherein the extreme pressure additive is 1,3-bis(9,10-epithiostearoyloxy)propane.

19. The composition of claim 15 wherein the extreme pressure additive is 2-ethoxyethyl 9,10-epithiostearate.

20. The composition of claim 15 wherein the extreme pressure additive is 2-(2-ethoxyethoxy)ethyl 9,10-epithiostearate.

21. The composition of claim 15 wherein the extreme pressure additive is 2-ethoxyphenyl 9,10-epithiostearate.

22. The composition of claim 15 wherein the extreme pressure additive is 4-methoxyphenyl 9,10-epithiostearate.

23. The composition of claim 15 wherein the extreme pressure additive is 1,3-bis(9,10-epithiostearoyl)-imidazolidine.

24. The composition of claim 15 wherein the extreme pressure additive is epithioated soybean oil.

25. The composition of claim 15 wherein the extreme pressure additive is 9,10-epithiostearyl 9,10-epithiostearate.

26. The composition of claim 15 wherein the extreme pressure additive is 9,10-epithiostearyl pentachlorostearate.

27. The composition of claim 15 wherein the extreme pressure additive is 9,10-epithiostearoyl terminated sebacic acid-1,3-propanediol polyester.

28. An extreme pressure lubricant composition wherein the base lubricant is a diester-base oil and the extreme pressure additive is selected from the group consisting of N-methyl-N-[2-(9,10-epithiostearoyloxy)ethyl]-9,10-epithiostearamide, N-[2-(9,10-epithiostearoyloxy)ethyl]-9,10-epithiostearamide, 1,3-bis(9,10-epithiostearoyloxy)propane, 1,3-di(9,10-epithiostearoyl) hexahydropyrimidine, 2-ethoxyethyl 9,10-epithiostearate, 2-(2-ethoxyethoxy)ethyl 9,10-epithiostearate, 2-ethoxyphenyl 9,10-epithiostearate, 4-methoxyphenyl 9,10-epithiostearate, 1,3-bis(9,10-epithiostearoyl)-imidazolidine, epithioated soybean oil, 9,10-epithiostearyl 9,10-epithiostearate, 9,10-epithiostearyl pentachlorostearate, and 9,10-epithiostearoyl terminated sebacic acid-1,3-propanediol polyester.

29. The composition of claim 28 wherein the extreme pressure component is N-methyl-N-[2-(9,10-epithiostearoyloxy)ethyl]-9,10-epithiostearamide.

30. The composition of claim 28 wherein the extreme pressure component is N-[2-(9,10-epithiostearoyloxy)ethyl]-9,10-epithiostearamide.

31. The composition of claim 28 wherein the extreme pressure component is 1,3-bis(9,10-epithiostearoyloxy)propane.

32. The composition of claim 28 wherein the extreme pressure component is 1,3-di(9,10-epithiostearoyl)-hexahydropyrimidine.

33. The composition of claim 28 wherein the extreme pressure component is 2-ethoxyethyl 9,10-epithiostearate.

34. The composition of claim 28 wherein the extreme pressure component is 2-(2-ethoxyethoxy)ethyl 9,10-epithiostearate.

35. The composition of claim 28 wherein the extreme pressure component is 2-ethoxyphenyl 9,10-epithiostearate.

36. The composition of claim 28 wherein the extreme pressure component is 4-methoxyphenyl 9,10-epithiostearate.

37. The composition of claim 28 wherein the extreme pressure component is 1,3-bis(9,10-epithiostearoyl)-imidazolidine.

38. The composition of claim 28 wherein the extreme pressure component is epithioated soybean oil.

39. The composition of claim 28 wherein the extreme pressure component is 9,10-epithiostearyl 9,10-epithiostearate.

40. The composition of claim 28 wherein the extreme pressure component is 9,10-epithiostearyl pentachlorostearate.

41. The composition of claim 28 wherein the extreme pressure component is 9,10-epithiostearoyl terminated sebacic acid-1,3-propanediol polyester.

\* \* \* \*

UNITED STATES PATENT OFFICE  
CERTIFICATE OF CORRECTION

PATENT NO. : 3,873,457

DATED : March 25, 1975

INVENTOR(S) : **Frank C. Magne, Robert R. Mod, Gene Sumrell and  
Winfred E. Parker**

It is certified that error appears in the above-identified patent and that said Letters Patent are hereby corrected as shown below:

[75] Inventors: **Frank C. Magne; Robert R. Mod;  
Gene Sumrell, all of New Orleans,  
La., and Winfred E. Parker, of  
Philadelphia, Pa.**

**Signed and Sealed this  
twenty-second Day of June 1976**

[SEAL]

*Attest:*

**RUTH C. MASON**  
*Attesting Officer*

**C. MARSHALL DANN**  
*Commissioner of Patents and Trademarks*